

UNITED STATES PATENT OFFICE

**2,237.096**

## LUBRICANT

**Frederick E. Dearborn, Washington, D. C.**

**No Drawing. Application September 22, 1939,  
Serial No. 296,096**

11 Claims. (Cl. 252—33)

(Granted under the act of March 3, 1883, as  
amended April 30, 1928; 370 O. G. 757.)

This application is made under the act of March 3, 1883, as amended by the act of April 30, 1928, and the invention herein described, if patented, may be manufactured and used by or for the Government of the United States of America for governmental purposes without the payment to me of any royalty thereon.

This application is a continuation in part of my application for patent Serial No. 189,961, filed February 11, 1938.

This invention relates to new compounds, useful as lubricant bases, prepared by reacting sulfurized unsaturated monocarboxylic acids with compounds of the class consisting of alkali salts, alkaline earth salts, and heavy metal salts.

The object of this invention is the provision of compounds suitable in compounding lubricants and greases for use under extreme pressure.

More specifically, the object is to provide a

similarly, the sulphur adding to the acid radical at the double bond. Animal and vegetable oils containing a large amount of the unsaturated acids may be used instead of the free acid. The amount of sulphur that may be chemically added to the unsaturated acid is dependent upon the number of double bonds in the acid molecule. For each double bond one atom of sulphur may be added to saturate that bond. Acids containing more than one double bond form a series of sulphurized acids, which are designated as the mono-, the di-, the tri-, etc., depending upon the number of double bonds saturated with sulphur. The following examples are given to illustrate the formation of these sulphurized acids.

### 1 *Oleic acid series*

Oleic acid contains only one double bond and hence can form only one sulphurized acid.



## 2. Linoleic acid series

Linoleic acid contains two double bonds in its molecule and combines with one or two atoms of sulphur forming the mono- and di- series of acids as shown by the following equations:



### 3. Linolenic acid series

Linolenic acid contains three double bonds in its molecule and combines with one, two, and

three atoms of sulphur, producing the corresponding sulphurized acids.

(a) Octadecadien-9, 12-monosulphur-oic acid.

EXAMPLE 1.—*Sodium salts of sulphurized linoleic acid*

(a) Sodium salt of octadecadien-9, 12-mono-



Linolenic acid

Sulphur

Octadecadien-9, 12-monosulphur-oic acid

(b) Octadecadien-9, 12-disulphur-oic acid.



Octadecadien-9, 12-disulphur-oic acid

(c) Octatrien-9, 12, 15-trisulphur-oic acid.



Octatrien-9, 12, 15-trisulphur-oic acid

The sulphurized monocarboxylic acids, whether mono-, di-, tri-, etc., react with alkalies forming the corresponding salts, which can be purified by repeated salting out from solution in a similar manner as used in the manufacture of soaps. A solution of these new alkali salts reacts with the alkaline earth and heavy metal salts, forming new alkaline earth and heavy metal compounds.

The preferred method of manufacturing these compounds is to heat a free unsaturated monocarboxylic acid with the appropriate amount of sulphur at a temperature ranging between 160-200° C., using iodine as a catalyst, until the sulphurized acids have been formed as shown by an exothermic reaction. An inert gas, such as carbon dioxide, is kept over the acid while heating and during the cooling process to prevent oxidation. Heating is preferably continued for half an hour or longer after the exothermic reaction stops to insure complete chemical reaction, and saturation of the double bond or bonds with sulphur. Glycerides of the unsaturated monocarboxylic acids, or animal and vegetable oils containing them, may be employed in place of the acids. The sulphurized acids are neutralized with a solution of sodium hydroxide, and purified by repeated salting out from solution. If a glyceride or oil has been sulfurized, it is saponified by digesting with sodium hydroxide solution, and then purified in the same way as outlined above. To form the alkaline earth and heavy metal salts the following procedure is used:

To a hot solution of the alkali salt of the sulphurized acid is added a hot solution of an alkaline earth or heavy metal salt, causing the precipitation of the corresponding sulphur compound. The compounds are well washed and dried. Most of the metallic salts of the sulphurized acids are amorphous compounds which are soluble in mineral oil on heating. They are partially soluble in organic solvents such as chloroform, benzene and other hydrocarbons. Typical examples of the formation of some of these new compounds are given below.

sulphur-oic acid.



(b) Sodium salt of octadecadien-9, 12-disulphur-oic acid.



EXAMPLE 2.—The sodium mono-, di-, and tri-compounds of sulphurized linoleic acid may be prepared as in the above example, using the formulas for the different acids previously described, by reacting one mole of the sulphurized acid with one mole of sodium hydroxide.

EXAMPLE 3.—*Lead salts of 9-10 monosulphur-octadecanoic acid*

This compound is prepared by reacting two moles of the corresponding sodium salt and one mole of a soluble lead salt.



**EXAMPLE 4.—Copper salts of octadecadien-9, 12-monosulphur-oic acid**

These two compounds are prepared by reacting two moles of the corresponding sodium salt with one mole of a soluble copper salt, producing the compounds



The copper compounds are green waxlike substances soluble in carbon tetrachloride, chloroform, and mineral oils when heated.

**EXAMPLE 5.—Tin salts of octadecadien-9, 12-monosulphur-oic acid and octadecadien-9, 12-disulphur-oic acid**

When two moles of a sodium salt of octadecadien-9, 12-monosulphur-oic acid or octadecadien-9, 12-disulphur-oic acid are reacted with one mole of a soluble tin salt the corresponding tin compounds of the formulas  $(\text{C}_{18}\text{H}_{31}\text{O}_2\text{S})_4\text{Sn}$  and  $(\text{C}_{18}\text{H}_{31}\text{O}_2\text{S}_2)_4\text{Sn}$  respectively, are formed. The tin compounds are yellowish white, puttylike substances soluble in mineral oils when heated.

**EXAMPLE 6.—Calcium salt of 9-10 monosulphur-octadecanoic acid**

When two moles of the sodium salt of 9-10 monosulphur-octadecanoic acid are reacted with one mole of a soluble calcium salt, the calcium salt of 9-10 monosulphur-octadecanoic acid is formed. This compound is of a yellowish white in color, amorphous in nature and forms an emulsion with mineral oils when heated. It has the general formula  $(\text{C}_{18}\text{H}_{33}\text{O}_2\text{S})_2\text{Ca}$ .

**EXAMPLE 7.—Magnesium salts of octadecadien-9, 12-monosulphur-oic and octadecadien-9, 12-disulphur-oic acid**

These two compounds are formed when two moles of the corresponding sodium salt are reacted with one mole of a soluble magnesium salt. The formulas of the two compounds are  $(\text{C}_{18}\text{H}_{31}\text{O}_2\text{S})_2\text{Mg}$  and  $(\text{C}_{18}\text{H}_{31}\text{O}_2\text{S}_2)_2\text{Mg}$  respectively. The compounds are amorphous and of a yellowish white in color. They form emulsions with mineral oils.

Having thus described my invention, I claim:

10. A lubricant containing in solution an alkaline earth salt of a sulphurized monocarboxylic acid to inhibit oxidation.
15. A lubricant containing in solution a heavy metal salt of a sulphurized monocarboxylic acid to inhibit oxidation.
20. A lubricant containing in solution a lead salt of 9-10-monosulphur-octadecanoic acid as an oxidation inhibitor.
25. A lubricant containing in solution a sodium salt of octadecadien-9, 12-monosulphur-oic acid as an oxidation inhibitor.
30. A lubricant containing in solution a sodium salt of octadecadien-9, 12-disulphur-oic acid to inhibit oxidation.
35. A lubricant containing in solution a sodium salt of octatrien-9, 12, 15-trisulphur-oic acid to inhibit oxidation.
40. A lubricant containing in solution a copper salt of octadecadien-9, 12-monosulphur-oic acid to inhibit oxidation.
45. A lubricant containing in solution a copper salt of octadecadien-9, 12-disulphur-oic acid to inhibit oxidation.
50. A lubricant containing in solution a magnesium salt of octadecadien-9, 12-monosulphur-oic acid to inhibit oxidation.
55. A lubricant containing in solution a magnesium salt of octadecadien-9, 12-disulphur-oic acid to inhibit oxidation.

FREDERICK E. DEARBORN.